

# UNITED STATES PATENT OFFICE.

CHARLES BITTNER, OF STAFFORD, KANSAS.

## PROCESS OF HARDENING AND WELDING COPPER.

1,122,062.

Specification of Letters Patent. Patented Dec. 22, 1914.

No Drawing.

Application filed June 6, 1914. Serial No. 843,514.

*To all whom it may concern:*

Be it known that I, CHARLES BITTNER, a citizen of the United States, residing at Stafford, in the county of Stafford and State of Kansas, have invented new and useful Improvements in Processes of Hardening and Welding Copper, of which the following is a specification.

My invention relates to a process of hardening and welding copper, the object of the invention being to provide a simple, reliable and efficient process, and compound employed therein, whereby copper may be quickly hardened to a material degree or rapidly welded while being hardened to make a strong joint.

In carrying my invention into practice, I employ a composition of acidified hyposulfite of soda, in crystal or granulated form or reduced to a powder. The said composition consists substantially of the following ingredients: Hyposulfite of soda, 16 ounces; sulfite of soda, 1/2 ounce; acetic acid No. 8 (containing 25% pure acid), 3 ounces; and powdered alum 1 ounce. These ingredients are thoroughly combined together in any suitable manner, and then reduced to a powder for use.

In employing the hardening compound, the piece of copper to be treated is heated in a forge or suitable flame to a good cherry heat. A little of the powder is then dusted on one side of the copper and allowed to fuse and burn off. The copper is then turned to present a fresh surface, on which a little of the powder is dusted in a similar manner and burnt off, and this operation is repeated, the copper being turned and the powder applied to the surfaces thereof, until the entire surface of the body of copper has been treated. In each instance the dusted surface is allowed to heat for a period of about thirty seconds, care being taken in order to prevent the use of too much of the compound at this stage, as it will tend to eat unduly into the copper. The copper is then, in a second stage of treatment, again treated in a similar manner, but at a low degree of heat or over a low fire, the compound being applied to the surface thereof and allowed to burn off until the entire surface of the copper is a second time treated. The copper at this stage is soft enough to be hammered or welded, and is then ham-

mered into the shape desired or welded and 55 then allowed to cool, when the process is completed.

By the process of treatment described, copper may be easily and conveniently hardened to a material degree. Copper so 60 treated will take an edge and be sufficiently hardened for cutting purposes, without tempering treatment of any kind. The acidified hyposulfite of soda in this composition acts mainly as the hardening agent, but its action 65 is promoted by the addition of the sulfite of soda and alum. Under some conditions the sulfite of soda and alum may be omitted, but their use is preferred, for the reason that more efficient results are obtained. 70

I claim:—

1. The herein described process of hardening copper, which consists in heating the copper to a cherry red, and then successively subjecting portions thereof to the 75 action of acidified hyposulfite of soda, until the whole of the surface of the copper is treated.

2. The herein described process of hardening copper, which consists in first heating 80 copper to a cherry red, successively treating portions of the heated copper at the cherry red temperature to the action of acidified hyposulfite of soda, and then repeating the above described treatment while the copper 85 is heated at a lower temperature.

3. The herein described process of hardening copper, which consists in heating the copper to a cherry red, and then successively subjecting portions thereof to the action of 90 hyposulfite of soda, acetic acid and alum, until the whole of the surface of the copper is treated.

4. The herein described process of hardening copper, which consists in heating the 95 copper to a cherry red, successively treating portions of the heated copper at the cherry red temperature to the action of a compound of hyposulfite of soda, acetic acid and alum, and then repeating the above described treatment while the copper is heated 100 at a lower temperature.

In testimony whereof I affix my signature in presence of two witnesses.

CHARLES BITTNER.

Witnesses:

JOHN A. BITTNER,  
F. B. HULL.